

Sept 17, 1957

J. JANSEN

2,806,267

CENTRIFUGAL CASTING MOLDS, ETC

Filed Feb. 14, 1957

2 Sheets-Sheet 1

Fig. 1



Fig. 2



Inventor:  
Johannes Jansen  
By Michael S. Striker

Sept 17, 1957

J. JANSEN

2,806,267

CENTRIFUGAL CASTING MOLDS, ETC

Filed Feb. 14, 1957

2 Sheets-Sheet 2



Inventor:  
Johannes Jansen  
By Michael S. Striker  
sp.

1

2,806,267

## CENTRIFUGAL CASTING MOLDS, ETC.

Johannes Jansen, Bochum, Germany, assignor to Bochumer Verein Fuer Gusstahlfabrikation Aktiengesellschaft, Bochum, Germany

Application February 14, 1957, Serial No. 640,101

12 Claims. (Cl. 22—113.5)

The present invention relates to centrifugal casting molds and processes for making the same.

This application is a continuation in part of my co-pending application Serial No. 314,292, filed October 11, 1952, and having the title "Centrifugal Casting Molds and Processes for Making the Same," now abandoned.

In the use of centrifugal casting molds, for making seamless cast iron pipe, for example, it is necessary for the molds to be cooled to permit continuous operation thereof. This cooling is usually provided in the form of a water jacket which is located about the outer surface of the turning mold. When one considers that the inner surface of such a mold, during use thereof, is placed at a temperature of 1100—1200° C., when molten gray cast iron is placed within the mold, it is apparent that the mold wall is subject to tremendous stresses. Because of the cooling of the outer surface of the mold, the heated inner surface thereof can only expand inwardly toward the axis of the mold and therefore this inner surface becomes upset. On the other hand, the metal of the mold is incapable of cooling quickly enough adjacent its inner surface to prevent the formation of cracks during the cooling of such a mold, and these cracks generally extend in the direction of the length of the mold. Such molds, which may have a wall thickness of 30—40 mm., cannot be used many times, and if a crack should unexpectedly occur during use of such a mold, the molten metal in the interior of the latter comes in contact with the cooling water and an explosion results.

One of the objects of the present invention is to overcome all of the above disadvantages by providing a centrifugal casting mold with an inner surface which is capable of expanding and contracting without causing undue stresses in the mold.

A further object of the present invention is to provide a centrifugal casting mold with an inner mold surface which is capable of expanding and contracting without damaging the mold and which at the same time presents a smooth inner surface to the molten metal being molded.

Another object of the present invention is to provide an inner surface portion of a centrifugal casting mold with a means for guaranteeing that the inner surface portion will retain its particular form despite expansion and contraction thereof.

An additional object of the present invention is to provide a process for inexpensively, efficiently, and simply manufacturing a centrifugal casting mold capable of accomplishing all of the above objects.

A still further object of the present invention is to provide a centrifugal casting mold which is capable of having only a damaged part thereof easily and quickly repaired or replaced without necessitating handling of undamaged parts of the mold.

With the above objects in view, the present invention mainly consists of an elongated, tubular, centrifugal casting mold having an inner surface portion formed with a plurality of grooves which are of a lesser width at the inner surface of the mold than immediately beneath said inner surface to form at said inner surface narrow gaps between their opposite edges, said gaps being adapted to

2

close due to thermal expansion of the areas between the grooves when the mold is heated during use thereof. These grooves may advantageously be formed on the inner surface of a lining which may take the form of a helically wound metallic band or of a plurality of metallic rings located next to each other.

Also with the above objects in view, the present invention mainly consists of a process for manufacturing a centrifugal casting mold, this process comprising the steps of forming in the interior surface portion of an elongated tubular mold a plurality of grooves, and applying pressure to the interior surface of this mold to narrow the grooves at this inner surface so as to produce a plurality of narrow gaps between their opposite edges, said gaps being adapted to close due to thermal expansion of the areas between the grooves when the inner surface is heated by a molten metal placed within the mold. This mold is advantageously formed from an outer casing into which a lining is placed, this lining having the grooves formed on the inner surface thereof before being placed within the casing.

The novel features which are considered as characteristic for the invention are set forth in particular in the appended claims. The invention itself, however, both as to its construction and its method of operation, together with additional objects and advantages thereof, will be best understood from the following description of specific embodiments when read in connection with the accompanying drawings, in which:

Fig. 1 is a fragmentary sectional view through an end portion of a centrifugal casting mold constructed in accordance with the present invention;

Fig. 2 is a fragmentary sectional view through a slightly different embodiment of a centrifugal casting mold constructed in accordance with the present invention;

Fig. 3 is a partly sectional, fragmentary view of still another embodiment of a centrifugal mold constructed in accordance with the present invention;

Fig. 4 is a fragmentary view of a part of the mold of Fig. 3 during the manufacture thereof;

Fig. 5 is a fragmentary view of a part of the structure of Fig. 4 taken along the line 5—5 of Fig. 4 in the direction of the arrows;

Fig. 6 is a fragmentary, sectional view of still another embodiment of a mold constructed in accordance with the present invention; and

Fig. 7 is a side view of one of the parts of the mold illustrated in Fig. 6.

Referring now to the drawings, there is shown in Fig. 1 a part of a mold having grooves 9 and 10 formed on the inner surface thereof. These grooves 9 and 10 intersect each other at angles of about 80° to 100° and are distributed over the inner surface of the mold. The grooves 9 and 10 are of a special construction in that they are narrower at the inner mold surface than immediately beneath this surface and thus form at the inner mold surface very narrow gaps between their opposite edges, said gaps being adapted to close due to thermal expansion of the areas between the grooves when the inner mold surface is heated during use of the mold. The narrower width of the grooves 9 and 10 at the inner surface of the mold may be produced by applying a pressure to the inner mold surface, preferably by cold working the latter so as to strengthen the material of the mold at this inner mold surface. This pressure may be produced by applying a roller or the like with a sufficient force against the inner mold surface or by pressing suitable dies or polishing instruments against the latter.

In order to make up for the loss of heat conductivity caused by the removal of material in cutting the grooves, and in order to fill the grooves so as to prevent the casting material from penetrating in its liquid state into the

grooves, a suitable insert material is placed within the grooves and the latter are narrowed about this insert. The insert preferably takes the form of a metal which has a high degree of heat conductivity and which is different from the metal of the inner mold surface.

Fig. 2 of the drawings shows a mold similar to that of Fig. 1 in that it includes grooves 9 and 10 of the same construction as the grooves of Fig. 1. The mold of Fig. 2, however, includes additional grooves 12 at a part of the molds where the diameter thereof changes so as to substantially prevent the formation of cracks at this critical part of the mold.

Fig. 3 of the drawings illustrates a mold which essentially differs from that of Figs. 1 and 2 in that the mold 13 carries on its inner surface a lining 14 formed with grooves 15 of the same construction as grooves 9, 10, and 12. It is of a particular advantage to provide such a lining on the interior of the mold 13, because it is much easier to form the grooves 15 on the lining before the latter is placed within the tubular mold 13 than it is to form grooves on the inner surface of a one-piece mold of the type shown in Figs. 1 and 2.

The lining 14 may be constructed in different ways. Thus, Fig. 4 shows the particular lining 14 of Fig. 3 during the manufacture thereof. This lining is formed from an elongated metal band which has the grooves 15 easily formed therein while the band is substantially flat as may be seen from the lower part of Fig. 4 and from Fig. 5. These grooves 15 extend transversely to the length of band 14. The band 14, which has the grooves 15 formed in only one side thereof, is helically wound with its successive convolutions located next to each other so as to form a cylinder which may be placed within the interior of the tubular member 13 either after the winding of band 14 or during the winding thereof. As may be seen from Fig. 4, the band 14 is wound so that the side thereof having grooves 15 therein is located on the inner surface of the cylindrical lining formed by the band 14, and Fig. 4 clearly illustrates how the grooves 15 are narrowed in this particular example by the winding of the band 14, this winding in itself producing a cold working on the inner surface of the lining which narrows the grooves 15 to produce very narrow gaps between their opposite edges on the inner surface of the mold. An insert 17, of a different material from band 14, is placed within the grooves 15 so that the latter are narrowed about the inserts 17 for the same purposes as set forth above in reference to Fig. 1. As is seen from Fig. 3, the lining 14 is located at one end thereof against a shoulder within the mold 13. The opposite end of the mold 13 may be threaded and may have an outwardly threaded ring engaging the threads on the interior of the mold 13 and abutting against the opposite end of lining 14 (not shown) to maintain the latter in its helically wound condition within the mold and guaranteeing that the lining fully covers the interior of member 13. A particular advantage of the lining 14 resides in the fact that stresses therein are distributed along its length which is quite long due to the helical winding.

The embodiment of Fig. 6 is identical in all respects with that of Fig. 3, except that the lining is formed by a plurality of identical rings 16 which are located against each other within the member 13 to form a lining therefor. One of the rings 16 is shown in the side view in Fig. 7, and it may be seen therefrom that the grooves 15 of ring 16 are identical with all of the above discussed grooves and extend transversely of the ring 16. The embodiment of Fig. 6 in addition to having the advantage of providing a means for easily manufacturing a mold having an inner grooved surface, has the additional advantage of permitting separate rings which happen to be damaged to be easily removed and replaced, so that undamaged parts of the mold may remain intact. The inner surface of the rings 16, before they are inserted into mold 13, are cold worked in any of the ways

described above to narrow the grooves 15 at the inner surface of rings 16.

It is to be understood that the insertion of heat-conductive material into the grooves is particularly useful if this material has a conductivity higher than that of the wall of the mold in the case of the embodiments illustrated by Figs. 1 and 2, or of the lining in the case of the embodiments shown by Figs. 3 to 7. In this manner, the removal of heat from the inner surface of the mold is substantially improved.

Various materials can be used as inserts. However, metal powders of high heat conductivity as for instance copper or aluminum have proven particularly satisfactory.

It is further to be noted that the automatic closing of the gaps between the opposite edges of the individual grooves at raised temperatures and the filling of the groove with a metallic insert material has the advantageous effect that the inner surface of the mold or its lining, respectively, presents during the casting operation to the liquid casting material a practically uninterrupted surface. If this were not the case, the pieces cast in the mold would form projections engaging existing gaps or grooves so that great difficulty would be encountered when the finished casting is to be pushed or pulled out of the mold.

The grooves referred to must be applied only to that inner zone of the mold or its lining which is exposed to the greatest extent to alternatingly changing temperatures. Considering conditions in molds of the type to which this invention is intended to be applied, the depth of the grooves is preferably chosen to be between  $\frac{5}{16}$ " and  $\frac{1}{2}$ ".

The mold proper may be made from any type of unalloyed or low-alloy steel. However, it is quite as well possible to make the mold of copper, aluminum or other metal provided that the material has sufficient ductility so that bursting of the mold is avoided.

The lining of the mold, as referred to in connection with the embodiments illustrated by Figs. 3 to 7, should be made of a material having great strength at high temperatures, which can be hardened to a tensile strength between 113,000 and 142,000 lbs./in.<sup>2</sup> and is suited for cold working.

As an example, a specific mold in accordance with the invention comprises an outside tubular member which may consist of low alloy or unalloyed steel. Its inner diameter may be 16", its outer diameter may be 18" and its overall length approximately 200". For the lining, a steel may be used which contains approximately .30% C, .60% Mn, .50% Si, 1.5% Cr, .5% Mo, and .3% V or .5% W. This material is rolled out as a strip with a cross-section of .8" thickness and 1.2" width. Grooves are cut into this strip by milling one narrow edge thereof, cutting into the material to a depth of about .39". The spacing between the individual grooves may be .8" and the width thereof may be .08". It is advisable to form the grooves with round corners at the bottom which prevents development of cracks in radial direction which would tend to start from sharp corners. After the strip is provided with the grooves it is helically wound around a mandrel having an outer diameter of 13.6", the grooved edge facing the mandrel. Therefore, the resulting coil has an outer diameter of 16" which corresponds to the inner diameter of the outer tubular member.

Before the strip is wrapped around the mandrel, the open grooves are filled with the insert material, for instance powdered copper. The granule size of this powder may vary between .0032" and .0315". After completion of the coil, the latter is subjected to the proper heat treatment while still held on the mandrel. During the heat treatment, not only the required tensile strength (113,000 to 142,000 lbs./in.<sup>2</sup> at room temperature) is obtained but at the same time the metal powder in the grooves is sintered. After tempering, the outer surface of the coiled strip is machined to exact dimension, if nec-

essary, for instance if there is a difference between the outer diameter of the coil and the inner diameter of the outer tubular member. After this, the coil is pushed into the tubular member and is attached to opposite ends of the mold by suitable means like screws, rivets, or even by welding, whereafter the mandrel can be forced out. Now, the lined mold is ready for machining the inner surface. The inner diameter may be increased by turning or grinding so as to increase the rough inner diameter by .039" to the desired final inner diameter. In this manner, after turning or grinding the inner surface, the depth of the individual grooves is approximately .315". Consequently, the finished mold has an inner diameter of 13.639" and an outer diameter of 18".

During the coiling operation, the shape of the originally straight grooves is changed because the edges of the grooves are forced towards each other, and at the same time the insert of metal powder is substantially compressed. It is to be noted that the reduction of the gap between opposite edges of a particular groove is not prevented by the presence of the metal powder. After machining the inside of the lining to finished dimensions, the inner surface appears as being entirely closed and free of gaps.

When the mold is first put to use, its inner zone expands considerably and causes compression of all the mold material exposed to the higher temperatures. Under these conditions, the opposing edges of the grooves are subjected to very high stresses due to the compression caused by thermal expansion. This condition exists as long as the inner surface of the mold is exposed to the prevailing temperatures. Under the influence of these pressure stresses the material has a tendency to creep which is due to the fact that the mold is continually exposed to certain changes in temperature. When the molten iron contacts the inner surface of the mold, it heats it up to high temperatures which, however, drop again rapidly soon thereafter. It is true that the temperature of the mold surface does not drop below a certain average temperature during continuous use of the mold, however conditions change entirely when the mold is taken out of service and cooled to room temperature. Under this condition the grooves do not remain tightly closed any more but open up depending upon the contraction of the surface area located between two consecutive grooves. It is within the scope of this invention to make these surface areas large enough in order to provide for ample "breathing" of the surface without risking too great an opening of the grooves when the mold finally cools down.

Whenever, at any times, the mold is put to use again, a rapid closing of the grooves before casting can be obtained by preheating the mold, for instance, with the aid of a gas or oil burner. However, this is not necessary if the inner surface is powdered with a silicon powder.

It will be understood that each of the elements described above, or two or more together, may also find a useful application in other types of centrifugal casting molds and processes for making the same differing from the types described above.

While the invention has been illustrated and described as embodied in centrifugal casting molds having removable liners and processes for making the same, it is not intended to be limited to the details shown, since various modifications and structural changes may be made without departing in any way from the spirit of the present invention.

Without further analysis, the foregoing will so fully reveal the gist of the present invention that others can by applying current knowledge readily adapt it for various applications without omitting features that, from the standpoint of prior art, fairly constitute essential characteristics of the generic or specific aspects of this invention and, therefore, such adaptations should and are intended

to be comprehended within the meaning and range of equivalence of the following claims.

What is claimed as new and desired to be secured by Letters Patent is:

5. An elongated, tubular centrifugal casting mold having an inner surface portion formed with a plurality of grooves which are of a lesser width at the inner surface of the mold than immediately beneath said inner surface to form at said inner surface narrow gaps between their opposite edges, said gaps being adapted to close when the mold is heated during use thereof; and heat-conductive means located in said grooves for keeping the edges of the latter, at the inner surface of the mold, apart from each other.
10. An elongated, tubular centrifugal casting mold having an inner surface portion formed with a plurality of grooves which are of a lesser width at the inner surface of the mold than immediately beneath said inner surface to form at said inner surface narrow gaps between their opposite edges, said gaps being adapted to close when the mold is heated during use thereof; and heat-conductive means located in said grooves for keeping the edges of the latter, at the inner surface of the mold, apart from each other.
15. An elongated, tubular centrifugal casting mold having an inner surface portion formed with a plurality of grooves which are of a lesser width at the inner surface of the mold than immediately beneath said inner surface to form at said inner surface narrow gaps between their opposite edges, said gaps being adapted to close when the mold is heated during use thereof; and heat-conductive means located in said grooves for keeping the edges of the latter, at the inner surface of the mold, apart from each other, said means being in the form of a metal different from the material of the mold and located within said grooves.
20. A process for manufacturing a centrifugal casting mold comprising the steps of forming in the inner surface portion of an elongated tubular mold a plurality of grooves; placing a pressure-resistant heat-conductive means within said grooves; and applying pressure to said inner surface to narrow said grooves about said pressure-resistant heat-conductive means so as to produce at said inner surface a plurality of narrow gaps between their opposite edges, said gaps being adapted to close when said inner surface is heated by a molten metal placed within the mold.
25. A centrifugal casting mold comprising, in combination, an elongated, rigid, tubular member; a lining located within said tubular member and against the same, said lining having its inner surface portion formed with a plurality of grooves which are of a lesser width at said inner surface of said lining than immediately beneath said inner surface of said lining so as to form at said inner surface of said lining a plurality of narrow gaps between their opposite edges, said gaps being adapted to close when the mold is heated during use thereof; and a heat-conductive metallic material located in said grooves.
30. A process for manufacturing a centrifugal casting mold, comprising the steps of forming a plurality of grooves on one side of an elongated band of metal; curving said band along a helix with the convolutions of the band located against each other, to form a tube from said band, and with said one side of said band forming the inner surface of said tube, so as to thereby cold work said inner surface to narrow said grooves at said inner surface; and placing said thus formed tube in the interior of a second tube and against the inner surface of the latter.
35. A process for manufacturing a centrifugal casting mold, comprising the steps of forming a plurality of grooves on one side of an elongated band of metal; curving said band along a helix with the convolutions of the band located against each other, to form a tube from said band, and with said one side of said band forming the inner surface of said tube, so as to thereby cold work said inner surface to narrow said grooves at said inner surface; and placing said thus formed tube in the interior of a second tube and against the inner surface of the latter.
40. A process for manufacturing a centrifugal casting mold, comprising the steps of forming on the inner surface of each of a plurality of identical rings a plurality of grooves; cold working the inner surface of each ring to narrow the grooves therein at the inner surface of each ring; and placing said rings next to each other within a rigid tubular member having an inner diameter substantially equal to the outer diameter of said rings, so that the latter form a lining on the interior of said tubular member.
45. A centrifugal casting mold comprising, in combination, an elongated, rigid, tubular member; and a lining located within said tubular member and against the same, said lining having its inner surface portion formed with a plurality of grooves and said lining being in the form of an elongated metallic band which is helically wound so as to form a cylinder.
50. A centrifugal casting mold comprising, in combination, an elongated, rigid, tubular member; and a lining located within said tubular member and against the same, said lining having its inner surface portion formed with a plurality of grooves and said lining being in the form of an elongated metallic band which is helically wound so as to form a cylinder.
55. A centrifugal casting mold comprising, in combination, an elongated, rigid, tubular member; and a lining located within said tubular member and against the same, said lining having its inner surface portion formed with a plurality of grooves and said lining being in the form of an elongated metallic band which is helically wound so as to form a cylinder.
60. A centrifugal casting mold comprising the steps of forming on the inner surface of each of a plurality of identical rings a plurality of grooves; cold working the inner surface of each ring to narrow the grooves therein at the inner surface of each ring; and placing said rings next to each other within a rigid tubular member having an inner diameter substantially equal to the outer diameter of said rings, so that the latter form a lining on the interior of said tubular member.
65. A centrifugal casting mold comprising, in combination, an elongated, rigid, tubular member; and a lining located within said tubular member and against the same, said lining having its inner surface portion formed with a plurality of grooves and said lining being in the form of an elongated metallic band which is helically wound so as to form a cylinder.
70. A centrifugal casting mold comprising, in combination, an elongated, rigid, tubular member; and a lining located within said tubular member and against the same, said lining having its inner surface portion formed with a plurality of grooves and said lining being in the form of an elongated metallic band which is helically wound so as to form a cylinder.
75. A centrifugal casting mold comprising, in combination,

tion; an elongated, rigid, tubular member; and a lining located within said tubular member and against the same, said lining having its inner surface portion formed with a plurality of grooves and said lining being in the form of a plurality of identical metallic rings located next to each other within said tubular member so as to form a cylinder.

9. A centrifugal casting mold comprising, in combination, an elongated, rigid, tubular member; and a lining located within said tubular member and against the same, said lining having its inner surface portion formed with a plurality of grooves and said lining being in the form of an elongated metallic band which is helically wound so as to form a cylinder, said grooves having a lesser width at the inner surface of said lining than immediately beneath said inner surface.

10. A centrifugal casting mold comprising, in combination, an elongated, rigid, tubular member; and a lining located within said tubular member and against the same, said lining having its inner surface portion formed with a plurality of grooves and said lining being in the form of a plurality of identical metallic rings located next to each other within said tubular member so as to form a cylinder, said grooves having a lesser width at the inner surface of said lining than immediately beneath said inner surface.

11. A centrifugal casting mold comprising, in combination, an elongated, rigid, tubular member; a lining located within said tubular member and against the same, said lining having its inner surface portion formed with a plurality of grooves and said lining being in the form of

an elongated metallic band which is helically wound so as to form a cylinder, said grooves having a lesser width at the inner surface of said lining than immediately beneath said inner surface; and an insert located within said grooves and being made of a material different from the material of said lining.

12. A centrifugal casting mold comprising, in combination, an elongated, rigid, tubular member; a lining located within said tubular member and against the same, said lining having its inner surface portion formed with a plurality of grooves and said lining being in the form of a plurality of identical metallic rings located next to each other within said tubular member so as to form a cylinder, said grooves having a lesser width at the inner surface of said lining than immediately beneath said inner surface; and an insert located within said grooves and being made of a material different from the material of said lining.

#### References Cited in the file of this patent

##### UNITED STATES PATENTS

|           |         |       |               |
|-----------|---------|-------|---------------|
| 609,460   | Peipers | ----- | Aug. 23, 1848 |
| 1,485,859 | Ladd    | ----- | Mar. 4, 1924  |
| 1,523,021 | Ladd    | ----- | Jan. 13, 1925 |
| 2,577,423 | Ludwig  | ----- | Dec. 4, 1951  |

##### FOREIGN PATENTS

|         |         |       |               |
|---------|---------|-------|---------------|
| 166,505 | Austria | ----- | Aug. 10, 1950 |
|---------|---------|-------|---------------|